

Patented Apr. 24, 1923.

1,453,254

# UNITED STATES PATENT OFFICE.

ALLEN B. NORTON, OF CLEVELAND, OHIO, ASSIGNOR TO ALUMINUM MANUFACTURERS, INCORPORATED, OF CLEVELAND, OHIO, A CORPORATION OF DELAWARE.

## ALLOY AND PROCESS OF MAKING THE SAME.

No Drawing.

Application filed May 31, 1921. Serial No. 473,826.

To all whom it may concern:

Be it known that I, ALLEN B. NORTON, a citizen of the United States, and a resident of Cleveland, county of Cuyahoga, State of Ohio, have invented certain new and useful Improvements in Alloys and Processes of Making the Same, of which the following is a specification.

This invention relates to metallic alloys and to processes of making the same. It is concerned particularly with aluminum alloys containing metals having relatively high melting points as compared with aluminum, and with a new and improved process by which they may be manufactured.

One object of the invention is to provide a new and improved alloy containing aluminum, copper and metals having higher melting points than aluminum and being substantially free from deleterious impurities.

Another object is to provide an aluminum alloy containing copper and other high melting point metals and being substantially free from aluminum oxide.

Another object of the invention is to provide a new and improved process of alloying aluminum with higher melting point metals.

Another object is to provide a new and improved process of producing an aluminum alloy containing copper and iron, each in amounts exceeding that ordinarily found in commercial aluminum.

Another object is to provide a process of producing alloys of the class described which may be practiced without arduous manual labor and without recourse to high temperatures or violent chemical or metallurgical reactions.

Other objects will be pointed out in the following specification.

My invention resides essentially in a new sequence of melting and alloying steps and in the new and unexpected advantages resulting therefrom. Heretofore, in making aluminum alloys containing metals having relatively high melting points as compared with aluminum, such as copper and iron, nickel, cobalt, manganese, chromium, or molybdenum, numerous difficulties and disadvantages have been encountered. In alloying, aluminum, copper and any one of these various high melting point metals it has been considered necessary, either to hold

the molten metal at a high temperature for a considerable period of time or to cause a thermit reaction in the molten copper or both in order to melt, dissolve or otherwise bring the high melting point metal into solution.

Holding aluminum or its alloys at high temperature for a considerable period of time has long been known to be harmful to the metal or alloy and is to be avoided whenever possible.

The thermit reaction requires that either, or both, of the high melting point metals be oxidized somewhat before the aluminum is added because it is the union of the aluminum with oxygen which brings about the intense heat and the solution of the solid metal in the liquid metals. Since certain oxides of copper are soluble in molten copper and also because of the brisk stirring accompanying the process, the aluminum oxide formed by the reaction is distributed throughout the bath and only part of it rises to the top from which it can be removed. Entrapped oxides are known to be harmful and it is believed that they form a frequent cause of porosity in aluminum alloy castings.

Furthermore, due to the high temperature and the presence of the various oxides, slag and other foreign materials in the bath, a tendency exists to the formation of small extremely hard particles which cannot be completely separated from the alloy and which are very destructive to sharp edged cutting tools employed in machining or finishing castings made from the alloy. A single particle will often damage a set of cutting tools to the extent of necessitating a replacement of the tools by sharp ones.

The making of an alloy containing aluminum and copper in nearly equal amounts and up to about 10% of iron will serve as illustrative of this general thermit process.

The copper and aluminum are first melted separately, the copper being melted in an open pot or furnace without any protection against oxidation. When the copper has been melted and raised to the proper temperature, iron, preferably in the form of annealed wire is added thereto, no effort being made to submerge the iron therein since some oxidation of the iron apparently promotes the subsequent thermit reaction. Molten aluminum is then poured into the

copper while the latter is briskly stirred, whereupon a violent thermit reaction takes place, part of the aluminum being oxidized by the copper and iron oxides and the remainder alloying with the copper and iron. This reaction raises the temperature of the bath considerably and effectually dissolves the iron and alloys it with the aluminum and copper.

10 The oxidized aluminum formed during the thermit reaction in part rises to the surface of the bath from which it is removed by skimming but considerable quantities remain entangled in the alloy and are carried 15 into the castings. Any small hard particles which are formed in the alloying process and which cannot be completely separated from the metal will appear in the castings.

The process is unduly costly first, because 20 the oxidized aluminum represents a considerable loss of metal and second, because the form of iron best suited to it is annealed wire which is more expensive than other forms, for example, scrap tin plate, turnings, 25 etc. Moreover, the resulting alloy is practically certain to contain aluminum oxide and may contain the hard substances previously referred to and an alloy made by adding aluminum to relatively small amounts of 30 an alloy containing such impurities will contain corresponding amounts of the impurities. In general it may be said that whenever these harmful impurities are formed in an alloy, they accompany it into whatever 35 combination of metals or kind of article the alloy may enter.

I have discovered, however, that such 40 metals as copper and iron, nickel, cobalt, manganese, chromium or molybdenum can be alloyed with aluminum by a simple process not involving arduous manual labor and without the aid of a thermit reaction and the 45 high temperatures and violent chemical or metallurgical reactions incident thereto.

45 The cheaper forms of iron of suitable compositions may be used. Such forms include scrap tin plate, clean, high grade, substantially pure iron or mild steel turnings, and in general any readily obtainable form 50 of suitable composition having a relatively large surface area as compared with its volume.

The solution of the iron in the copper and 55 aluminum is brought about in a manner to prevent a violent thermit reaction. Probably not more than inappreciable amounts of aluminum oxide are formed in the alloying step of the process. Consequently, castings made from such alloys are substantially free 60 both from porosity due to entrapped aluminum oxide and from hard particles. Furthermore, the aluminum lost thru oxidation is reduced to the small amount which unavoidably forms during the melting of the

metal. The cost of the process is thus correspondingly decreased and at the same time a more nearly uniform product is obtained due to the small unvarying amount of aluminum oxidized by the process.

65 My improved process, as applicable to the previously enumerated metals is typified by the following detailed description of its use in connection with an aluminum, copper, iron alloy.

70 In the manufacture of an alloy containing aluminum 50%, copper 40% or more and iron up to about 10%, I first melt the calculated amount of aluminum and maintain it at a temperature slightly above the melting point, preferably not above 1400° F. Simultaneous therewith the calculated amount of copper is melted and raised to a 75 temperature slightly above the melting point but preferably not above 2200° F. When both metals have been brought to the desired temperature, the calculated amount of iron is introduced into and submerged in the molten aluminum. The copper is then 80 poured into the aluminum while the latter is gently stirred or agitated. The iron goes into solution quickly and easily without much increase in temperature and without the violent reactions common to the thermit reaction, and, as soon as all the copper has 85 been added, the finished, homogenous alloy 90 is ready for casting, further alloying or treating as may be desired.

95 For purposes of illustrating my process and the resulting alloys I have particularly 100 specified aluminum, copper and iron each in certain amounts which have been found suitable. It is obvious, however, that the 105 amounts may vary greatly without affecting the steps of the process and, accordingly, I do not wish to be understood as limiting myself to the specified percentages of these 110 constituent metals. Nor do I wish to be limited to these three metals since so far as adaptability of my process is concerned 115 many other metals may be the equivalent of iron. Among such equivalents may be included nickel, cobalt, manganese, chromium and molybdenum, all of which are to be considered as within the limits of my invention. 120 Altho my experiments have not been exhaustive they prove that such metals may replace iron in my improved process, the 125 amounts of the metals which actually enter the alloy, however, being dependent on a 130 number of factors such as solubilities, melting temperatures, etc., as will be understood by those skilled in the art.

135 The scope of my invention is defined by what is claimed.

What is claimed:

1. The process of making an alloy containing aluminum and metals having relatively high melting points as compared with

aluminum, which comprises melting the aluminum, adding a high melting point metal in solid form to the molten aluminum and then adding a high melting point metal in 5 molten form to the molten aluminum.

2. The process of making an alloy containing aluminum, copper and a metal having a melting point higher than that of aluminum, which comprises adding the last 10 mentioned metals in solid form to the molten aluminum and introducing the copper in molten form into the aluminum.

3. The process of making an alloy containing aluminum, copper and iron which 15 comprises adding molten copper to a bath of molten aluminum containing unmelted iron, and stirring the molten bath until the iron has alloyed with the copper and aluminum.

20 4. The process of making an alloy containing aluminum, copper and iron which comprises melting the aluminum and copper separately, adding iron in sheet form to the molten aluminum and then adding the 25 molten copper to the molten aluminum.

5. The process of making an alloy containing aluminum, copper and iron, the aluminum and copper being present in pre- 30 ponderating amounts which comprises melting the aluminum and bringing it to a temperature slightly above its melting point, melting the copper and bringing it to a temperature slightly above its melting point, adding iron in sheet form to the molten alu- 35 minum, and then pouring the molten copper into the molten aluminum whereby the iron becomes alloyed with the copper and aluminum.

6. The process of making an alloy con-

taining aluminum, copper and iron which 40 comprises melting the aluminum and maintaining it at a temperature of about 1400° F., adding iron thereto in solid form, melting the copper and maintaining it at a temperature of about 2200° F. and then causing so- 45 lution of the iron, at temperature below 2000° F. by introducing the molten copper into the aluminum with stirring.

7. The process of making an alloy containing aluminum, copper and iron which 50 comprises melting the aluminum and copper separately, then adding the iron in solid form to the aluminum and then alloying the iron with the aluminum and copper by adding the latter to the aluminum bath in a 55 manner to prevent substantial oxidation of the aluminum.

8. The process of making an alloy containing aluminum, copper and iron which 60 comprises melting the aluminum and copper separately, adding iron in solid form to the aluminum, and then bringing about the so- 65 lution of the iron and the alloying thereof with the aluminum and copper by addition of the latter in a manner to prevent the formation of hard particles in the finished alloy.

9. A metallic alloy comprising aluminum, copper and a metal having a high melting point as compared with aluminum, charac- 70 terized by being substantially free from aluminum oxide.

10. A metallic alloy containing aluminum, copper and iron characterized by being sub- 75 stantially free from aluminum oxide.

In testimony whereof I affix my signature.

ALLEN B. NORTON.